

March 15, 1932

S. RUBEN

1,849,157

INSULATING COATING FOR FILAMENTS

Filed Sept. 23, 1929



INVENTOR  
SAMUEL RUBEN  
BY  
Chester W. Braselton  
ATTORNEY

## UNITED STATES PATENT OFFICE

SAMUEL RUBEN, OF NEW YORK, N. Y., ASSIGNOR TO RUBEN TUBE COMPANY, OF ENGLEWOOD, NEW JERSEY, A CORPORATION OF DELAWARE

## INSULATING COATING FOR FILAMENTS

Application filed September 23, 1929. Serial No. 394,850.

This invention relates to heater type vacuum tubes, and particularly to an insulating coating for the filamentary heaters of such tubes.

5 One of the objects of the invention is to produce a coating for the heater of a heater type vacuum tube which is capable of withstanding a large potential difference between the heater and a contacting cathode without 10 leakage or electrolysis at the normal operating temperatures.

Another object of the invention is to provide a heater coating which has a low vapor pressure and high melting point, so that it 15 will not volatilize during operation of the tube in which it is used and thereby cause a change in its insulating qualities.

Another object of the invention is to provide a heater coating which may be heated 20 to a temperature much higher than that to be used in the normal operation of the heater to permit complete degasification.

A further object of the invention is to provide a heater coating which may be handled, 25 bent, and stored for future use without chipping or cracking or otherwise deteriorating.

Another object of the invention is to provide a graded coating for a vacuum tube heater which is capable of fusing to the heater material at the point of contact but presents a fine grained insulating outer surface. 30

Still another object of the invention is to provide a heater coating which is extremely 35 dense and heat conductive and which is integral with the resistance material of the heater to give a minimum temperature gradient in the coating itself and a minimum thermal lag.

Other objects of the invention will be apparent as the description thereof proceeds.

In connection with the drawings,

Fig. 1 is a view in elevation of a section of a radio tube embodying my invention; and

Fig. 2 is a detail of one of the heater cathode units.

The compounds of certain metals are valuable as insulators, and of these compounds the lower the atomic number of the metal element the higher the specific resistance and 50 the higher the temperature at which the in-

sulating qualities are maintained. In other words, compounds of barium, calcium, cadmium, strontium, and zinc lose their insulating qualities and become conductive at relatively low temperatures while compounds of boron, magnesium, aluminum, silicon and beryllium have insulating characteristics at much higher temperatures, such temperatures varying substantially inversely in each group to the atomic numbers. Beryllium and magnesium having the lowest numbers, the compounds have the highest specific resistance and may be heated to extremely high temperatures without decomposing or losing their insulating qualities. Beryllium is better in this respect than magnesium, and for use on the filaments of vacuum tubes, therefore, where high temperatures are required, I prefer to use the compounds of beryllium, although I do not wish to limit myself to this particular metal.

To attain the objects of the invention I have found it necessary to provide a graded coating with a base layer next to the resistance wire which will fuse to the wire at temperatures very much higher than normal operating temperatures and which will therefore act as a bonding agent between the resistance wire and an outer insulating layer with which it is adapted to have a slight chemical reaction so as to closely bind the two together. This outer layer must be highly refractory and of high specific resistance at the maximum operating temperature.

The inner or base layer of the coating may be made by mixing finely ground beryllium aluminosilicate ( $3\text{BeO} \cdot \text{Al}_2\text{O}_3 \cdot 6\text{SiO}_2$ ) with ammonium borate ( $\text{NH}_4\text{B}_2\text{O}_7$ ) in the proportion by weight of three of beryllium aluminosilicate to one of ammonium borate with enough water to give proper consistency. The beryllium aluminosilicate should be ground fine enough to fall through a size 250 screen mesh. This mixture is coated upon the resistance wire, which may be of tungsten or other desirable material, and a current of about 1.5 amperes is then passed through the wire to heat it and dry the coating in place. I have found it preferable to apply two coats of this material to form the

inner layer of the insulating coating, although more layers may be added if found desirable. Two coats make the thickness approximately .01 of a millimeter.

5 The outer layer is preferably made of beryllium oxide ( $Be_2O_3$ ). The coating material for this oxide is prepared by grinding the oxide in a ball mill with 25% by weight of ammonium borate and enough distilled water to give the desired consistency. The mixture is then applied to the filament carrying the intermediate coating of beryllium aluminosilicate. This application is made cold and the coated filament then heated to 10 about 500° C. at which temperature the ammonium borate decomposes—forming ammonia gas, water vapor and boric oxide. At 15 least five successive coatings of the beryllium oxide material should be applied. The successive heatings during the coating process also cause a partial sintering of the coating material.

20 The wire thus provided with its insulating coating may be handled and bent, and welded in position in a vacuum tube, the coating having enough flexibility so that it will not crack or chip off.

25 If the wire is not to be used at once, preferably it should receive a thin collodion coating so as to avoid moisture absorption by the coating. This coating may best be applied by placing the wire in a vessel containing a solution of collodion and allowing the wire to remain in the solution until the occluded gas 30 escapes, being displaced by the collodion which then forms an adherent skin layer. Water absorption may also be avoided by subjecting the coating to a high temperature so as to vitrify the material thereof, but such 35 treatment makes the coating more or less brittle and should be used preferably only when the filament is formed prior to heating.

40 When properly placed in the vacuum tube, the tube may be exhausted in the ordinary manner. To do this it is necessary to raise the temperature of the filament a great deal higher than it is heated in normal operation of the tube the temperature in some instances reaching as high as 2000° C. At this temperature the first or inner layer of beryllium aluminosilicate will fuse with the resistance wire and form a dense, hard, flexible coating which is substantially integral with the wire. The beryllium oxide, however, which forms 45 the outer layer or surface of the insulating coating will withstand temperatures in the neighborhood of 2400° C. without melting, and, therefore, is not affected by the high temperature used in exhausting the tube. At 50 the exhausting temperature all physically or chemically unstable components of the coating are discharged, so that the resistance wire and coating may be completely degasified. There is, however, a slight chemical action 55 between the inner and outer layers which

firmly knits the two together, making a substantially integral structure.

60 The drawings illustrate an application of the invention to the heater cathode of a radio tube, in which 10 is the envelope, 11 the plate, 12 the grid, 13 the cathode, and 14 the heater filament. The filament 15 is illustrated as provided with a coating 16 which may at intervals contact with the cathode 13. When used on a filament maintained at the proper 65 operating temperature, this coating has been found to have no leakage or electrical conductivity when potentials up to 80 volts have been placed between the filament and the contacting cathode, but to readily conduct heat from the filament to the cathode with a minimum of time lag. If the tube has been 70 evacuated the coating on the filament is absolutely stable, and as it has been completely 75 degasified, will not cause any deterioration 80 of the operation or efficiency of the tube, but 85 will protect the filament and greatly add to its life.

90 While beryllium oxide has highly desirable characteristics as an external coating and is used as a preferable material, I have found that aluminum oxide may be mixed with the beryllium oxide up to a limit of 75% by weight of aluminum oxide, without destroying 95 the effectiveness of the coating.

100 As indicated above, still other materials may be used in the insulating coating, and I do not therefore desire to limit the invention to any specific material except as defined in the appended claims.

105 Having thus described my invention, what I claim is:

1. A heater cathode unit for a radio tube of the heater type comprising a refractory heater filament, a plurality of superimposed coatings containing beryllium oxide on said filament, and a tubular cathode enclosing and in approximate contact with said superimposed coatings.

110 2. A heater cathode unit for radio tubes of the heater type comprising a refractory heater filament, a coating containing beryllium oxide on said filament, a binder coating having a chemical affinity for the first mentioned coating, and a cathode tube enclosing and in approximate contact with said coating.

115 3. A heater cathode unit for radio tubes of the heater type comprising a refractory heater filament, a coating of beryllium aluminosilicate on said filament, a second coating containing beryllium oxide on said first named coating, and a cathode tube enclosing and in approximate contact with said coating.

120 4. A heater unit for a heater type radio tube comprising a refractory filament, a binder coating containing beryllium, a coating of beryllium oxide having a chemical affinity for the binder coating.

5. In a heater type radio tube, a heater cathode unit comprising a filamentary heater element, a coating on said heater containing an oxide of the magnesium group which is normally substantially non-conductive at operating heater temperature, and the binder coating interposed between the first mentioned coating and the heater, said binder coating also containing an oxide of the magnesium group.

10 6. A heater cathode unit for a heater type radio tube comprising a filamentary heater, an oxide of an element having a low atomic number which is normally substantially non-conducting at normal operating temperatures of the tube heater and which possesses a vapor pressure less than that of tungsten, and a binder coating between said oxide and the heater, said binder also including an element having a low atomic number and having an affinity for the said oxide.

15 7. In a radio tube of the heater type, a heater cathode unit comprising a heater filament, a coating of beryllium oxide on said filament, and a bonding coating intermediate said coating of beryllium oxide and the filament, the melting point of the elements of the bonding coating being less than that of the beryllium oxide, whereby an intimate, 20 dense, and highly heat conducting layer is formed intermediate the beryllium oxide and said filament, and a cathode enclosing and external to said beryllium oxide coating.

25 In testimony whereof, I affix my signature.  
35 SAMUEL RUBEN.

40

45

50

55

60